

## 1

3,075,838

## MANGANESE STEEL

Howard S. Avery and Henry J. Chapin, Mahwah, N.J.,  
assignors to American Brake Shoe Company, New 5  
York, N.Y., a corporation of Delaware  
No Drawing. Filed Feb. 24, 1960, Ser. No. 10,557  
2 Claims. (Cl. 75—123)

This invention relates to manganese steel and in particular to a standard 13% manganese steel so alloyed as to be capable of effective precipitation hardening resulting in yield strength values of better than 70,000 p.s.i. and elongation of at least about 10%. This represents, in comparison to the standard heat treated alloy, a significant enhancement in yield strength achieved at a sacrifice in elongation which is not deemed detrimental for many uses.

Manganese steel is well known for the ease with which it can be work hardened. Precipitation hardening is not commonly followed. The practice, where followed, has been to solution heat treat at about 2000° F. followed by a quench or rapid cool to hold a metastable-austenitic structure. This preliminary step is the standard heat treatment for manganese steels as the mode of achieving maximum toughness. After this, the casing is aged at a temperature substantially under 2000° F. to precipitate a hardening phase, but the associated loss in toughness attendant to such precipitation hardening procedure is usually too great to warrant general adoption. While the role of vanadium has heretofore been recognized in precipitation hardening, we have now found that the above specified values of yield strength and elongation can be attained in a precipitation hardened manganese steel by combining vanadium with nickel, or nickel and molybdenum, provided that the carbon content does not exceed about 0.7%; in fact, superior results are achieved by holding carbon within the narrow range of 0.4–0.5%; and furthermore, we have found that vanadium is so potent in increasing yield strength at a sacrifice of lowered ductility in a standard 13% manganese steel that its content should be restricted to not more than about 0.9% in conjunction with the aforesaid carbon limitation; and so to do is the primary object of this invention. Another object of the present invention is to so restrict the hardening treatment as to assure the desired results.

Exceptional results are achieved by limiting carbon to 0.4–0.5% and vanadium to 0.7–0.9%. The significance of this lowered carbon content can be best appreciated by realizing that carbon is usually specified as about ten percent of the manganese level which would therefore be about 1.2–1.4% for a standard 13% manganese steel. This combination, together with about 2% each of nickel and molybdenum in a standard 13–14% manganese steel ("standard 13%") produces, after precipitation hardening, a yield strength of 90–100,000 p.s.i. and an elongation of 20–30%. This in comparison to the standard toughened alloy represents a doubling of yield at a sacrifice at the outside of only about half the ductility, and the accomplishment of this is another object of the present invention.

## 2

This preferred alloy can vary as follows:

| C, Percent | Mn, Percent | Si, Percent | Ni, Percent | Mo, Percent | V, Percent | P, Percent | S, Percent |
|------------|-------------|-------------|-------------|-------------|------------|------------|------------|
| 0.4        | 13.7        | 0.2         | 1.7         | 1.9         | 0.7        | 0.04       | 0.04       |
| 0.5        | 14.3        | 0.8         | 2.3         | 2.1         | 0.9        | Max.       | Max.       |

10 Typical of an alloy within this narrow range is heat "24" hereinafter which in round figures is 0.5% C, 14% Mn, 2% Ni, 2% Mo and 0.8% V. Following the conventional or standard toughening treatment (2000° F.—2 hours—water quench), to provide standard manganese steel properties, aging at 1080° F. for 8 hours hardened alloy "24" to 262 BHN, raised yield to 95,640 p.s.i. and lowered elongation to 29.5%. Aging at 1200° F. for 2 hours gave a higher hardness (277 BHN), a yield of 99,300 and 21.5% elongation. Eight hours at 1200° F. raised the yield, but elongation was unacceptable at 9.5%. Aging at 1300° F. and 1400° F. for 6 hours also lowered ductility too far.

15 20 The following table sets forth data pertinent to three alloys that represent the outside limits of carbon (0.7%) and vanadium (about 0.3%) under the present invention:

TABLE I

| Heat | C, Percent | Mn, Percent | Si, Percent | Ni, Percent | Cr, Percent | Mo, Percent | V, Percent | Al, Percent |
|------|------------|-------------|-------------|-------------|-------------|-------------|------------|-------------|
| 348  | 0.70       | 13.90       | 0.44        | 6.02        | -----       | -----       | 0.56       | 0.085       |
| 342  | 0.70       | 13.94       | 0.46        | 3.00        | -----       | -----       | 0.49       | 0.064       |
| 218  | 0.52       | 13.75       | 0.42        | 2.08        | -----       | 2.12        | 0.28       | 0.015       |

## AS CAST

| Heat | Yield <sup>1</sup> | Tensile <sup>2</sup> | Elong. <sup>3</sup> | R.A. <sup>4</sup> | BHN |
|------|--------------------|----------------------|---------------------|-------------------|-----|
| 348  | 49.2               | 88.7                 | 27.5                | 33.4              | 156 |
| 342  | 49.2               | 79.4                 | 21.0                | 29.5              | 170 |
| 218  | 49.3               | 101.7                | 36.0                | 34.1              | 207 |

## TOUGHENED BY 2,000° F., 2 HOURS, WATER QUENCH (W.Q.)

| Heat | 44.2 | 105.9 | 67.0 | 47.6 | 163 |
|------|------|-------|------|------|-----|
| 348  | 45.2 | 109.9 | 55.5 | 42.5 | 143 |
| 342  | 47.6 | 109.1 | 61.5 | 50.0 | 174 |

## HARDENED BY 1,200° F., 2 HOURS, W.Q. (AFTER TOUGHENING)

| Heat | 71.4 | 105.7 | 27.5 | 28.8 | 207 |
|------|------|-------|------|------|-----|
| 348  | 65.8 | 95.9  | 22.0 | 23.7 | 228 |
| 342  | 64.1 | 114.2 | 44.0 | 35.4 | 192 |

## HARDENED BY 1,250° F., 2 HOURS, W.Q. (AFTER TOUGHENING)

| Heat | 84.5 | 104.9 | 15.0 | 27.2 | 241 |
|------|------|-------|------|------|-----|
| 348  | 73.8 | 111.9 | 27.5 | 28.9 | 235 |

## HARDENED BY 1,300° F., 2 HOURS, W.Q. (AFTER TOUGHENING)

| Heat | 82.2 | 106.9 | 18.0 | 26.8 | 241 |
|------|------|-------|------|------|-----|
| 342  | 74.2 | 108.7 | 24.5 | 28.9 | 223 |

## HARDENED BY 1,300° F., 6 HOURS, W.Q. (AFTER TOUGHENING)

|                                           | Heat No. | YS <sup>1</sup>                              | TS <sup>2</sup> | Elong. <sup>3</sup> | R.A. <sup>4</sup> | BHN | Thermal history, °F., hours cooling |
|-------------------------------------------|----------|----------------------------------------------|-----------------|---------------------|-------------------|-----|-------------------------------------|
| 348                                       | 5        | 57.6                                         | 107.2           | 30.0                | 29.8              | 180 | As cast.                            |
| 342                                       |          | 50.6                                         | 115.8           | 59.0                | 44.0              | 174 | 2000-2-WQ.                          |
| 218 <sup>5</sup>                          | 21...    | 3.5                                          | 141.5           | 14.0                | 17.0              | 286 | 2000-2-WQ+1400-6-WQ.                |
|                                           |          | 12.3                                         | 154.0           | 10.0                | 15.2              | 332 | 2000-2-WQ+1300-6-WQ.                |
|                                           |          | 30.5                                         | 148.5           | 13.5                | 16.6              | 321 | 2000-2-WQ+1300-2-WQ.                |
|                                           |          | 33.0                                         | 140.0           | 20.5                | 20.2              | 286 | 2000-2-WQ+1200-8-WQ.                |
| HARDENED BY 1,300° F., 12 HOURS, AIR COOL |          |                                              |                 |                     |                   |     |                                     |
| 218 <sup>5</sup>                          | 10 24... | 81.6                                         | 128             | 18.5                | 23.4              | 277 |                                     |
|                                           |          | 1. P.s.i. $\times 10^3$ based on 0.2% set.   |                 |                     |                   |     |                                     |
|                                           |          | 2. P.s.i. $\times 10^3$ .                    |                 |                     |                   |     |                                     |
|                                           |          | 3. Percent in 2".                            |                 |                     |                   |     |                                     |
|                                           |          | 4. Percent.                                  |                 |                     |                   |     |                                     |
|                                           |          | 5. Requirements of yield and elongation met. |                 |                     |                   |     |                                     |

The values for yield, tensile, elongation and reduction in area in Tables II and III which follow are on the same bases as noted above in the footnotes of Table I.

In view of our observation that high carbon contents (above about 0.7%) have a drastic effect in lowering ductility, it was concluded that the best combination of enhanced yield and not seriously impaired elongation would be found at even lower carbon levels, provided carbon was not so low as to require having resort to sources of expensive manganese, as distinguished from ferromanganese, and more expensive alloying in general. Nickel, for instance, is expensive and desirably is held to a minimum for this reason. The following heats, therefore, represent the preferred and least expensive form of alloy practices under the present invention, and it should be mentioned that it was these heats that lead to the above set forth range for the preferred alloy:

TABLE II  
Precipitation Hardenable Manganese Steels  
With 0.4% Carbon

| Heat No. | Chemical composition |             |             |             |             |             |            |            |
|----------|----------------------|-------------|-------------|-------------|-------------|-------------|------------|------------|
|          | C, percent           | Mn, percent | Si, percent | Cr, percent | Ni, percent | Mo, percent | V, percent | P, percent |
| 28       | 0.40                 | 13.90       | 0.48        | 4.04        | 2.03        | 0.90        | 0.04       | 0.045      |
| 29       | 0.39                 | 14.22       | 0.52        | 2.08        | 4.08        | 2.03        | 0.90       | Max: 0.053 |
| 37       | 0.42                 | 14.20       | 0.48        | 3.93        | 3.55        | -----       | 0.90       | 0.066      |

| Heat No. | Yield <sup>1</sup> | Tensile <sup>2</sup> | Elong. <sup>3</sup> | R.A. <sup>4</sup> | BHN | Thermal history, °F., hours cooling |
|----------|--------------------|----------------------|---------------------|-------------------|-----|-------------------------------------|
| 28       | 54.7               | 96.1                 | 23.0                | 28.6              | 196 | As cast.                            |
|          | 48.6               | 105.5                | 48.5                | 37.3              | 174 | 2000-2-WQ.                          |
|          | 82.2               | 132.0                | 13.5                | 17.8              | 283 | 2000-2-WQ+1400-6-WQ.                |
|          | 106.2              | 143.0                | 7.5                 | 12.2              | 332 | 2000-2-WQ+1300-6-WQ.                |
|          | 5110.1             | 143.0                | 10.0                | 11.8              | 332 | 2000-2-WQ+1300-2-WQ.                |
|          | 5107.5             | 132.5                | 17.5                | 23.3              | 262 | 2000-2-WQ+1200-8-WQ.                |
|          | 5108.3             | 133.0                | 21.5                | 27.8              | 286 | 2000-2-WQ+1200-4-WQ.                |
| 29       | 56.0               | 98.2                 | 27.5                | 31.6              | 207 | As cast.                            |
|          | 49.6               | 102.0                | 44.0                | 34.4              | 228 | 2000-2-WQ.                          |
|          | 5181.9             | 133.0                | 13.5                | 17.0              | 286 | 2000-2-WQ+1400-6-WQ.                |
|          | 110.4              | 147.0                | 8.5                 | 12.2              | 332 | 2000-2-WQ+1300-6-WQ.                |
|          | 112.1              | 145.0                | 9.5                 | 13.4              | 302 | 2000-2-WQ+1300-2-WQ.                |
|          | 5199.0             | 127.5                | 21.0                | 29.8              | 293 | 2000-2-WQ+1200-8-WQ.                |
|          | 5104.8             | 131.0                | 23.5                | 26.8              | 277 | 2000-2-WQ+1200-4-WQ.                |
| 37       | 55.4               | 103.2                | 31.5                | 31.5              | 196 | As cast.                            |
|          | 48.2               | 106.1                | 46.0                | 37.5              | 183 | 2000-2-WQ.                          |
|          | 5186.5             | 138.0                | 14.0                | 15.2              | 170 | 2000-2-WQ+1400-6-WQ.                |
|          | 5101.0             | 144.0                | 11.0                | 14.5              | 302 | 2000-2-WQ+1300-6-WQ.                |
|          | 5191.4             | 119.6                | 18.5                | 23.2              | 270 | 2000-2-WQ+1200-8-WQ.                |

See footnotes, Table I.

TABLE III  
Precipitation Hardenable Manganese Steels  
With 0.5 Carbon

| Heat No. | Chemical composition |             |             |             |             |             |            |            |
|----------|----------------------|-------------|-------------|-------------|-------------|-------------|------------|------------|
|          | C, percent           | Mn, percent | Si, percent | Cr, percent | Ni, percent | Mo, percent | V, percent | P, percent |
| 21       | 0.50                 | 14.05       | 0.54        | -----       | 2.06        | 2.04        | 0.55       | 0.04       |
| 24       | 0.50                 | 13.82       | 0.49        | -----       | 2.08        | 2.07        | 0.83       | Max: 0.051 |
| 26       | 0.49                 | 14.10       | 0.60        | 2.11        | 2.08        | 2.07        | 0.81       | -----      |

See footnotes, Table I.

It will be seen from the foregoing that under the present invention, we are able to increase significantly, by precipitation hardening, the yield strength in a standard 13% manganese steel without seriously impairing ductility. This is accomplished by holding carbon between the limits of about 0.4-0.7%, preferably 0.4-0.5% for the best balance of yield and elongation, and holding vanadium to between about 0.3-0.9%. It is moreover important to observe that precipitation hardening can be accomplished efficiently and at low cost because in several instances the hardening is produced after only two to four hours of heat treatment.

The alloy is further characterized by nickel contents of about 2 to 6%. Thus, nickel can be as low as about 2% provided about 2% of molybdenum is present, but 3% nickel (heat 342; also note heat 37) produces satisfactory results with molybdenum absent. From this and other data we have concluded that the present alloy should contain at least 3% total of nickel and molybdenum.

Hence, while we have illustrated and described preferred embodiments of the present invention, it is to be understood that these are capable of variation and modification, and we therefore do not wish to be limited to the precise details set forth, but desire to avail ourselves of such changes and alterations as fall within the purview of the following claims.

We claim:

1. An austenitic manganese steel alloy containing about 13 to 14% manganese capable of being precipitation hardened to produce a yield strength of 70,000 p.s.i. (0.2% set) and an elongation of at least 10% (in 2") and containing carbon restricted to the range of about 0.4 to 0.7%, vanadium additions restricted to the range of about 0.3 to 0.9%, and an addition selected from the group consisting of (a) about 3 to 6% nickel and (b) at least 2% each of nickel and molybdenum up to a total nickel-molybdenum content of about 6%, balance essentially iron.

2. An alloy according to claim 1 wherein carbon is restricted to the narrow range of 0.4-0.5% carbon, having a yield strength of 90-100,000 p.s.i. (0.2% set) and an elongation of at least about 20% (in 2"), after precipitation hardening.

References Cited in the file of this patent

UNITED STATES PATENTS

2,865,740 Heger et al. Dec. 23, 1958

OTHER REFERENCES

Bullens: Steel and Its Heat Treatment, vol. 2, 4th ed., page 406, published by John Wiley & Sons, Inc., New York, N.Y.